

A. E. VANDERCOOK.  
PROCESS OF EXTRACTING PRECIOUS METALS FROM THEIR ORES.  
APPLICATION FILED OCT. 24, 1914.  
1,198,086. Patented Sept. 12, 1916.



WITNESSES:

*J. G. Frost*  
*J. B. Gaudus*

INVENTOR.  
A. E. VANDERCOOK.  
BY *White & Frost*  
his ATTORNEYS.

# UNITED STATES PATENT OFFICE.

ALBERT E. VANDERCOOK, OF ALAMEDA, CALIFORNIA, ASSIGNOR OF ONE-HALF TO  
LESLIE B. McMURTRY, OF SAN FRANCISCO, CALIFORNIA.

## PROCESS OF EXTRACTING PRECIOUS METALS FROM THEIR ORES.

1,198,086.

Specification of Letters Patent. Patented Sept. 12, 1916.

Application filed October 24, 1914. Serial No. 868,459.

To all whom it may concern:

Be it known that I, ALBERT E. VANDERCOOK, a citizen of the United States, and a resident of Alameda, county of Alameda, 5 and State of California, have invented a certain new and useful Process of Extracting Precious Metals from Their Ores, of which the following is a specification.

The invention relates to amalgamation in 10 cyanid solution.

An object of the invention is to render amalgamation in cyanid solution practical.

Amalgamation in cyanid has been practised in several ways heretofore, but either 15 the results obtained have been such as to discourage the use of such step or the cost thereof has been excessive. In spite of the recognized advantages of amalgamation in removing the coarser metallic particles of 20 gold and silver upon which the dissolving effect of cyanid is slow, owing to the great disadvantages of the usual amalgamation practise, when crushing in solution, amalgamation is not largely practised. There is 25 always a mechanical loss of mercury and of amalgam from the plates which finds its way into the tailings.

Another object of the invention is to provide a process by which the alkali sulfids are 30 automatically removed from the cyanid solution as quickly as they are formed or by which their formation in the solution is prevented. The sulfur of the sulfid minerals of the ores enters into solution in working cyanid 35 solutions and produces alkali sulfids. The deleterious effect of alkali sulfids is well known. They are powerful reducing agents and cyanicides and cause the precipitation of dissolved silver, as silver sulfid, and 40 may under certain conditions re-precipitate gold and silver. In ordinary practice, soluble lead salts, such as lead acetate, are added to the solution to combine with the alkali sulfids and form lead sulfids, which are precipitated. This practice however, is not subject to any exact control and is governed by 45 experience or guess, with the result that too much or too little soluble lead salts are

added. The results obtained are comparatively erratic.

In the present process, the alkali sulfids are removed from the solution as quickly as they form, and the sulfur is precipitated in the form of mercuric sulfid. Mercury is, of course, always present in any amalgamating process, and in my process the amount of mercury which enters the solution is just sufficient to produce the desired reaction and form the insoluble mercuric sulfid, which is precipitated.

A further object of the invention is to dispose of the use of metallic copper in amalgamation practice. The deleterious action of copper on cyanid solution is well known. Its presence occasions a consumption of cyanid, a consumption of copper, a reducing action, a consumption of zinc in the precipitating apparatus or devices and the introduction of copper into the precipitates and bullion.

A further object of the invention is to provide an amalgamating process in which the mercury is maintained in a bright and active condition and is prevented from fouling, sickening or flowering.

The invention possesses many other advantageous features, some of which, with the foregoing, will be set forth at length in the following description, where I shall outline in full one specific form of the process of my invention.

In the accompanying drawings I have shown one specific form of apparatus which may be employed in carrying out the process. I shall describe only one specific form 85 of my generic invention, but it is to be understood that I do not limit myself to such form because my invention may be embodied in a multiplicity of forms, each being a species of my said invention.

It is also to be understood that by the claims succeeding the description of my invention I desire to cover the invention in whatever form it may be embodied.

Referring to said drawings: Figure 1 is a 95 vertical section of one form of apparatus

with which my invention may be practised. Fig. 2 is a top or plan view of the apparatus.

Before entering upon a description of the process, I shall briefly describe the apparatus illustrated. The apparatus consists of a tank or receptacle 2, preferably formed of wood, in the bottom of which is arranged an iron pan 3, having standing edges. In this pan is placed a quantity of mercury. Arranged above the pan and out of contact with the pan and the mercury therein is an agitator, which is rotatably mounted upon the depending conductor 4. The agitator consists of the central gland or receptacle 5 which is provided with hollow arms 6, each arm being provided with a plurality of inclined nozzles 17. The agitator is rotated by the reaction of the liquid discharging from said nozzles, and the inclination of the nozzles is such that the discharging liquid is directed against the surface of the mercury.

The liquid or slimes or pulp which is discharged from the nozzles is taken from the tank through the pipe 7 and forced by the centrifugal pump 8 through the pipe 9 and down through the conductor 4. Fresh liquid or slimes carrying metallic particles to be amalgamated is fed into the tank through the pipe 12. In order to insure these particles being brought into intimate contact with the mercury and thereby hastening their amalgamation, the pipes 12 and 7 are so arranged that all material entering through pipe 12 is drawn into pipe 7 and hence is conveyed to the agitator. The pipes 7 and 12 are preferably joined by a  $\text{T}$  13, the third socket of which is open, thereby allowing the liquid or slimes in the tank to be drawn into the pump. This arrangement causes the particles of metal to be discharged against the mercury a plurality of times, and thereby increases the extraction by amalgamation. The agitation and circulation of the solution also assists greatly in effecting the solution of the metallic particles in the cyanid solution. The tank is provided with an overflow pipe 14 for the value bearing cyanid solution and with a discharge pipe 15. The suction pipe 7 is preferably provided with an air cock 16, so that when desirable air may be admitted to the solution.

By providing an iron pan to hold the mercury, all of the deleterious effects produced by the presence of copper are eliminated. The agitator and the various conductors and pipes which are in contact with the cyanid solution are also made of iron. When two different metals are placed in cyanid solution, a galvanic couple is formed, and if the metals are connected by a metallic conductor, an electric current will flow through the conductor and through the so-

lution. The effect of this current through the solution when mercury is used as one of the metals, is to cause a sickening and flowering of the mercury which greatly reduces its ability to amalgamate. This is one of the reasons why amalgamation in cyanid solution has not proved very successful in the past. In carrying out the process of my invention I suspend the agitator above and out of contact with the mercury, so that the galvanic couple is not completed. There is, therefore, no electric current passing through the solution, and hence the mercury remains bright and active.

Alkali sulfids are always formed in cyanid practice when the ore contains sulfid minerals and these minerals are present in a great proportion of gold and silver ores. These alkali sulfids are very deleterious and must be removed, and their removal heretofore has generally been accomplished by the addition of soluble lead salts, such as lead acetate. This lead salt combined with the alkali sulfid to produce insoluble lead sulfid, which precipitated. There has been no practical method of determining the proper amount of lead salts to employ in a given working condition, and consequently too much and too little have been used. I have found that mercury is soluble in cyanid solution, producing a double cyanid of mercury and potassium or sodium, and that the solubility is effected by the presence of oxygen, which either enters directly into the reaction or combines with evolved hydrogen, removing it from occlusion so that the reaction may proceed. One equation giving the reaction is as follows:



The presence of oxygen is essential. The amount of mercury going into solution in a given time is controlled by the amount of oxygen available. There may be sufficient air dissolved in the solution to produce the desired reaction, but it is advisable to provide means for introducing air in controllable amounts so that sufficient of the double cyanid may be formed. Silver and gold are readily soluble in the double cyanid, the precious metals displacing the mercury, which precipitates. In practice the double cyanid appears to possess greater silver dissolving properties than the single cyanid. The double cyanid also attacks the alkali sulfids as soon as they are formed or as they are forming, and causes a precipitation of the sulfur as mercuric sulfid, as



Just enough of the double cyanid is consumed as is necessary to remove the alkali sulfids from the solution. The remaining

double cyanid acts as a solvent for the gold and silver, and precipitates mercury as a result of the displacement of the mercury by the gold and silver.



The lead salts which have been heretofore used to remove the alkali sulfids have no solvent action on the precious metals and 10 their presence is rather deleterious. The necessary and uncertain excess of lead salt are lost as the sulfate and carbonate and serve no useful purpose.

In the present process, a slight trace of 15 mercury is found on the zincs under normal working conditions. The double cyanid of mercury and potassium or sodium performs its functions as it is formed and does not accumulate in the solution. The consumption 20 of mercury is very slight and the cost of consumed mercury per ton of ore treated is insignificant. This process produces the amalgamation of the metallic particles of gold and silver under conditions of marked 25 efficiency and by the solution of the mercury in cyanid forming mercuric cyanid a powerful aid in the dissolution of the gold and silver is obtained, and the alkaline sulfids are desulfurized at the moment of formation. An excess of mercuric cyanid is not 30 deleterious since the double cyanid possesses marked dissolving properties, taking up the gold and silver and precipitating the mercury. An automatic balance in the solution 35 is maintained.

In carrying out the process, a quantity of mercury is poured into the iron pan and the 40 slimes or mixture of cyanid solution and ground ore is fed into the tank. When sufficient slimes have accumulated in the tank to submerge the pump suction pipe, the 45 pump is started and the liquid becomes thoroughly agitated and the metallic particles are brought into intimate and recurring contact with the mercury. Since the agitator is out of electrical contact with the 50 mercury or with the iron pan, no current flows through the electrolyte, and hence the deleterious effect of the current, which is present in almost all other forms of amalgamators, is not encountered. Due to the 55 presence of air, either in solution or admitted, the double cyanid of mercury and potassium or sodium is formed. The double cyanid 60 acts as a solvent for the gold and silver and also attacks and removes the alkali sulfids. The metallic particles in the ore either become amalgamated or are dissolved by the cyanid solution. The values are recovered from the value bearing cyanid solution in the usual manner by precipitation 65 and are removed from the amalgam by retorting or otherwise. The presence of the slight amount of mercuric cyanid in the so-

lution as it is delivered to the precipitating apparatus aids in the precipitation of the precious metals. Presumably the mercury forms a galvanic couple with the zinc, which aids the precipitation. The presence of the mercuric cyanid also retards the precipitation of copper if this metal is present in the solution.

I claim:

1. The process of recovering precious metals from a mixture of sulfid ore and metallic particles with a sodium or potassium cyanid solution, which consists in agitating the mixture in the presence of mercury whereby a double cyanid of mercury and sodium or potassium is formed which 70 removes the alkali sulfids from the solution.

2. The process of recovering precious metals from a mixture of sulfid ore and metallic particles with a sodium or potassium cyanid solution, which consists in 80 bringing the mixture into recurrent impinging contact with mercury and in forming in the solution a double cyanid of mercury and sodium or potassium.

3. The process of recovering precious 90 metals from a mixture of sulfid ore and metallic particles with a sodium or potassium cyanid solution, which consists in agitating the mixture in the presence of mercury and oxygen whereby some of the metallic particles become amalgamated and some become dissolved by the solution.

4. The process of amalgamating metallic particles in a cyanid solution, which consists in directing a plurality of streams of 100 the mixture against mercury while maintaining the stream directing means out of electrical contact with the mercury.

5. The process of recovering precious metals from sulfid ores containing the same, 105 which consists in mixing the ground ore with cyanid solution whereby the finer metallic particles are dissolved, bringing the mixture into contact with metallic mercury whereby the larger metallic particles are 110 amalgamated and whereby a double cyanid of mercury and sodium or potassium is formed which combines with the alkali sulfids formed in the solution and causes a precipitation of the sulfur content of the alkali sulfids, separating the solution from the metallic mercury and precipitating the values in the solution.

6. The process of recovering precious 120 metals from sodium or potassium cyanid solutions containing the same in solution and in a metallic state and sulfid ore particles which consists in bringing the mixture into contact with metallic mercury whereby the precious metallic particles are amalgamated 125 and whereby the double cyanid of mercury and sodium or potassium is formed which causes a precipitation of the sulfur content

of the alkali sulfids in the solution as insoluble mercuric sulfid and separating the solution from the metallic mercury.

7. The process of amalgamating metallic particles in a cyanid solution containing the same and sulfid ore particles which produce alkali sulfids in the solution, which consists in bringing the mixture into contact with metallic mercury whereby the particles are 10 amalgamated and a double cyanid of mer-

cury and potassium or sodium are formed which removes the alkali sulfids from the solution.

In testimony whereof, I have hereunto set my hand at San Francisco, California, this 15 13th day of October 1914.

ALBERT E. VANDERCOOK.

In presence of—  
H. G. PROST,  
M. L. CONTE.